

## UNITED STATES PATENT OFFICE

2,191,037

COLOR FORMING DEVELOPER CONTAINING  
AMINES

Leopold D. Mannes and Leopold Godowsky, Jr.,  
Rochester, N. Y., assignors to Eastman Kodak  
Company, Rochester, N. Y., a corporation of  
New Jersey

No Drawing. Application November 12, 1938,  
Serial No. 240,048

3 Claims. (Cl. 95—88)

This invention relates to color photography and particularly to a method for developing multi-layer film.

In certain processes of multi-color photography, it is necessary to develop simultaneously several emulsion layers carried on one side of the support. In these processes the developer must penetrate all of the layers and develop an image in the innermost layer in about the same time as that required to develop an image in the outer layer, as otherwise the outer layer will be over-developed and too dense. A process of this type is described in our prior Patent 2,113,329, granted April 5, 1938. As described therein, a multi-layer film after exposure and reversal is subjected to a color-forming development which produces a blue-green dye and a metallic silver image in each of three superposed emulsion layers. In this process the developer is required to penetrate the three emulsion layers and develop an image in each of the layers, and it is desirable for the developer to penetrate and form the image as rapidly as possible.

It is, therefore, an object of the present invention to provide a photographic developer for multi-layer film having an increased rate of penetration of the emulsion layers. A further object is to provide a method for developing colored images in multi-layer film in shorter time than was hitherto possible. Other objects will appear from the following description of our invention.

These objects are accomplished by adding a primary aliphatic amine, such as ethylene diamine, to a color-forming developer in which a primary aromatic amine, such as diethyl para-phenylene diamine or a para-amino phenol, is used as the developing agent.

In developing multi-layer film, such as that described in our prior Patent 2,113,329, in color-forming developers to produce colored images in the layers, the developing agent used is a primary aromatic amino compound, such as para-dimethyl amino aniline, 2-amino-5-diethyl amino toluene, or para-amino phenol. If the three layers of the film are to be developed first to silver and a blue-green dye, the developing solution may contain a phenolic or naphtholic coupling compound, such as a chlorinated phenol, 2:4 dichloro alpha naphthol or other unsubstituted or substituted naphthol, or a dihydroxy naphthol such as 1:5-dihydroxy naphthalene. For reasons of dye stability it is desirable to choose certain couplers in preference to others and the phenolic or naphtholic cou-

plers are frequently desirable for this reason, although they do not penetrate the emulsion layers as rapidly as is desired. An alkaline developing solution containing these compounds develops the upper layer with ease, but develops the bottom layer only after an excessively prolonged immersion.

We have found that by adding to the coupler developers described above a primary aliphatic amine, such as methylamine, ethylamine, or ethylene diamine, the developing time of these developing solutions is considerably decreased and the bottom emulsion layer readily developed. In many cases the aliphatic amines, besides increasing the rate of penetration, have an additional beneficial effect in retarding deposition of a general dye fog, thereby improving the character of the dye image. These compounds may also prevent excessive surface development, thereby insuring more even dye formation throughout the thickness of the emulsion layers.

A suitable formula for a rapidly penetrating color-forming developer is as follows, it being understood that this example is merely illustrative.

|                                   |                   |      |
|-----------------------------------|-------------------|------|
| 2-amino-5-diethylamino toluene    | grams             | 2.5  |
| Sodium sulfite                    | do                | 20   |
| Sodium sulfate                    | do                | 40   |
| Sodium carbonate                  | do                | 40   |
| Potassium bromide                 | do                | 2 30 |
| Ethylene diamine                  | do                | 3    |
| Ammonium hydroxide (28% solution) |                   |      |
|                                   | cubic centimeters | 2    |
| 2:4 dichloro- $\alpha$ -naphthol  | gram              | 1    |
| Water to                          | liter             | 1 35 |

The above developer, without the ethylene diamine, develops a multi-layer film of the type described in our prior Patent 2,113,329 in about twenty minutes. When the ethylene diamine is added to the developer, the developing time is decreased to about 12 minutes. With color-forming developers containing from one to five grams of developing agent per liter of developing solution, the amount of ethylene diamine or other organic amine may vary from about one gram to about five grams.

The use of organic amines such as ethylene diamine has previously been suggested for black and white photographic developers, but as far as we are aware there has been no previous suggestion of the use of these compounds in color developers, particularly color-forming developers of the type containing a primary aromatic amino developing agent and a coupler compound for

the purpose of increasing the rate of penetration of multi-layer by the developer.

It is to be understood that the examples and modifications referred to in the above specification are illustrative only and that our invention is to be taken as limited only by the scope of the appended claims.

We claim:

1. A color-forming photographic developer 10 having a rapid rate of penetration for gelatin layers, comprising a primary aromatic amino developing agent, a compound which couples with the oxidation product of the developing agent on photographic development, and a primary 15 aliphatic amine.

2. A color-forming photographic developer

having a rapid rate of penetration for gelatin layers, comprising a primary aromatic amino developing agent, a compound which couples with the oxidation product of the developing agent on photographic development, and ethylene 5 diamine.

3. A color-forming photographic developer having a rapid rate of penetration for gelatin layers comprising a dialkyl amino aniline developing agent, a compound which couples with 10 the oxidation product of the developing agent on photographic development, and ethylene diamine.

LEOPOLD D. MANNES.

LEOPOLD GODOWSKY, JR. 15